

# UNITED STATES PATENT OFFICE.

ROBERT FULTON TOMPKINS, OF NEW YORK, N. Y., ASSIGNOR TO THE BINDER COMPANY, A CORPORATION OF NEW JERSEY.

## COHERING OR BINDING COMPOSITION AND PROCESS OF MAKING THE SAME.

1,171,905.

Specification of Letters Patent.

Patented Feb. 15, 1916.

No Drawing. Application filed August 11, 1913, Serial No. 784,121. Renewed August 4, 1915. Serial No. 43,707.

*To all whom it may concern:*

Be it known that I, ROBERT FULTON TOMPKINS, a citizen of the United States, residing at New York city, in the county of New York and State of New York, have invented certain new and useful Improvements in Cohering or Binding Compositions and Processes of Making the Same, of which the following is a specification.

10 This invention relates to binding compositions for substances of divided or separated nature, such as sand or insoluble silicious or silicon containing material, or other substance of mineral, vegetable, or animal nature, and process of making same.

The object of the invention is to provide an efficient binder of vegetable nature or carbon compound character comprising a glucosid, or tannin and glucosid associated 20 with water, or water and soluble silicates, such as sodium silicate, and has for certain specific applications the property of binding, securing or anchoring road-dust together in such a manner that its circulation 25 by air currents occasioned by moving vehicles or other means is limited or prevented and whereby a solid compact and hardened road-bed and road dressing is produced and an automatic hydroscopic coherence or adhesion created, without materially injuring 30 or destroying the coherer or adhering binder, and also for binding molder's sand or compositions for cores, etc., for gluing, sizing, or cementing of cellular or cellulose containing material or products or fabrications 35 thereof, such as paper, paste-board, straw board, and the like, and for other purposes.

One species of the composition included in the present invention comprises glucosids of 40 the aromatic extractive type, such as glucosid tannins which appear in tanning extracts or products, in proportion of about 27% by weight together with tannin 21% and water 52%, which composition has an 45 approximate gravity of forty-eight degrees Twaddell. This product or composition may be produced by concentrating the spent tan liquors containing approximately 2% of glucosid and tannin in approximate proportion to each other by weight as one and a half to one, or an aqueous solution of 2% Twaddell, by evaporation or 50 dehydration to a density of 48 degrees

Twaddell. To this aqueous solution of glucosid and tannin is preferably added a soluble silicate such as sodium silicate, in proportion of 5% by weight of the combined glucosid and tannin content when the binder is intended to be employed as a street or road dressing or as a cement or glue for 60 paper, straw or other cellulose containing substances or fabrications.

The advantages of this binder, comprising glucosids and tannin resides in the fact that when applied to paper or other cellulose substances which are matted or bonded by glues or sizes of glue nature, that the glucosid tannins and other tannins act as a glue or binder while they simultaneously fix the glue or size bonding material in the 70 paper or other cellulose fabrication making a practically water repelling seal or binding, while the glucosid present is just sufficiently hygroscopic to prevent the drying out of the material to a point of brittleness thus producing a substantially water-repellent and flexible or resilient gluing medium. The soluble sodium silicate, when employed, also augments the adhering of the composition 75 and maintains a flexibility which does not occur when substances comprising the silicate alone, as in the prior art, are employed.

When the binder is employed as a road dressing or binder, the tannin or tannic acid combines with the iron, alumina, lime or other constituents of the road construction material producing water insoluble compounds which present to the glucosids and other ingredients of the binder a superior adhesive surface so that the glucosids and excess tannins act as an agglutinating agent 80 for anchoring or securing particles of dust or other material together in a fixed and flexible or elastic manner while the inherent hygroscopic properties of the glucosids provide a ready and automatic moistening constituent and effect without deliquescence so that the particles adhere together without becoming attached to foreign materials 85 which may contact with them such as vehicle tires, etc., employed in the construction.

The glucosids employed may be of any 90 selective character, they being compounds which combine the properties of glucose and vegetable extractives, or what may be 95 termed glucose esters, in such a manner that

each has lost its specific physical identity as such and is less soluble than either individually in water as a rule, and is hygroscopic without deliquesence and does not effloresce 5 or dry up spontaneously. The peculiarly adaptable properties or qualities of these glucosids probably is attributable to a progressive and alternate hydrolysis into vegetable extractives or organic or carbon containing acids and glucose and its reformation of glucosids by condensation and dehydration under atmospheric conditions of heat, moisture, and pressure. The soluble silicate, such as sodium silicate, augments the 10 cementing and anchoring qualities of the composition especially when associated with insoluble silicates, silicious, or silicon containing substances such as are usually found associated with or form a part of road construction. The composite composition of these ingredients associated with water therefore produces a peculiarly advantageous material of selective utility as a cement or binder of flexible resilient, and elastic 15 nature in character.

Any glucosid associated with tannin may be employed and mixed in any selective or desired proportion without departing from the spirit of the invention, so long as both 20 are present in some form or the glucosid in itself presents and exhibits the combined properties hereinbefore set forth.

The soluble silicate, such as sodium silicate, may be employed as a binder augmenting 25 agent or additive constituent of the composition to modify the properties thereof with reference to its silicious cementing character and also for the purpose of resinsifying some of the tannins and converting 30 them into more water repellent substances.

The composition of tannin and glucosids may be produced by mixing the individual 35 ingredients with water or secured from such substances as spent tan liquors, or from other sources, or extracted from natural 40 derivatives, or artificially or synthetically prepared. Some of the tannins and tannic acids are at once so called tannins and glucosids, they being converted by hydrolysis 45 into glucose and gallic, ellagic, protocatechuic and other acids or organic extractives.

The composition comprising glucosids and tannins together with water, such as may be obtained from or as spent tan liquors, or 50 fluid tan waste products such as are ordinarily thrown away, either as such or products which may be obtained by boiling down or concentrating the same, or such concentrated product rediluted, is particularly 55 adaptable to road treatment, acting as it does to fix the dust and cement the road base thus maintaining a form of fixed binder which is continually working its way into 60 and between particles or pieces of the road construction when subjected at intervals to

progressive watering either by artificial sprinkling or from the natural source of rain, etc., and exhibits the further enhancing quality of presenting a latent form of moisture by reason of its hygroscopic properties 70 thus preventing the disintegration and drying out or crumbling of the road dressing or base body, and also provides a superior dressing or binding agent for construction materials of roads or other solid vehicle or transportation bearing body or path. This material applied to the surface of such roads as asphalt roads or pathways, and then coated or sanded with frictionable substances, has the property of anchoring or securing such 75 material to the asphalt surface thereby preventing the slipping of horses or skidding of vehicle wheels, the astringent properties of the tannin ingredients augmenting the frictional surface of the road as presented 80 to contacting substances such as vehicle tires, and also presents the additional feature of holding and securing or anchoring frost and ice to the roadway in such a manner that it is not easily released under pressure and 85 forms a foothold of frictional character for horses' shoes and the like, thus avoiding the usual dangerous character presented when ice is formed upon water repellent surfaces such as asphalt, which results in slipping 90 under pressure through the release of the unanchored ice coating.

The preferred process whereby this composition is made for employment as a road or roadway dressing, is to secure or provide a 100 spent tan liquor from a tannery or other source which averages in density approximately two degrees Twaddell or about two per cent. of soluble content comprising tannin and glucosids in proportion of about one of the former to one and a half of the latter by weight; this spent tan liquor is then exposed to the action of heat either by direct means or through the medium of circulating air at a higher temperature than the liquor and 105 preferably under reduced pressure whereby the vaporization of the aqueous content or evaporation of the material is facilitated. This drying or dehydrating action is continued until the fluid or liquor has been concentrated to about forty-eight degrees Twaddell or approximately 48% of the 110 tannin and glucosid. This concentration to 48 degrees Twaddell is made in order to facilitate the preservation of the liquor from decomposition and to cheapen and facilitate 115 shipment to points where it is to be utilized. This concentrated liquor is then diluted with water in the locality where it is to be employed in proportion of one part of concentrated liquor to three parts of water for a first coating or sprinkling of a road or roadway and one part to two parts of water for a second or final coating or sprinkling. 120 This dust cohering and roadway cementing 125 130

fluid has the advantage over oil dressings in that it does not injure or destroy rubber tires of vehicles or affect the varnish of the same injuriously, nor is it lost by evaporation, nor does it affect injuriously, metal, wood or leather, or reduce the gravity of the road dressing so that it is floated and washed away by water or give a greasy appearance or dull coating to varnish or contents of vehicles.

Having now described my invention what I claim as new and desire to secure by Letters Patent is:—

1. A cohering or binding composition comprising a glucosid, a tannin and a soluble silicate.
2. A cohering or binding composition comprising a glucosid, a tannin, a soluble silicate and water.
3. A cohering or binding composition comprising an aromatic glucosid, a tannin and a soluble silicate.
4. A cohering or binding composition comprising an aromatic glucosid, a tannin, a soluble silicate and water.
5. A cohering or binding composition comprising a glucosid, a tannin and sodium silicate.
6. A cohering or binding composition comprising a glucosid, a tannin, sodium silicate and water.
7. A cohering or binding composition comprising an aromatic glucosid, a tannin and sodium silicate.
8. A cohering or binding composition comprising an aromatic glucosid, a tannin, sodium silicate and water.
9. A cohering or binding composition

comprising the constituents of spent tan liquor.

10. A cohering or binding composition comprising the constituents of spent tan liquor and a soluble silicate.

11. A cohering or binding composition comprising the constituents of spent tan liquor and sodium silicate.

12. A cohering or binding composition comprising the concentrated or dehydrated constituents of spent tan liquor.

13. A cohering or binding composition comprising the concentrated or dehydrated constituents of spent tan liquor and a soluble silicate.

14. A cohering or binding composition comprising the concentrated or dehydrated constituents of spent tan liquor and sodium silicate.

15. The process of making a cohering or binding composition which comprises subjecting a spent tan liquor to the action of heat and removing the vapors evolved.

16. The process of making a cohering or binding composition which comprises subjecting a spent tan liquor to the action of heat under reduced pressure and removing the vapors evolved.

17. The process of making a cohering or binding composition which comprises dehydrating a spent tan liquor.

In testimony whereof I affix my signature in presence of two witnesses.

ROBERT FULTON TOMPKINS. [L. s.]

Witnesses:

WM. J. JULIEN,  
JOHN HENRY HURLBUTT.